

# UNITED STATES PATENT OFFICE.

AUSTIN GILBERT AND CHARLES E. VANDER HOOF, OF HAMILTON, OHIO, ASSIGNORS TO  
THE FISCHER CAN COMPANY, OF HAMILTON, OHIO.

## SEALING COMPOSITION FOR CANS.

1,323,752.

Specification of Letters Patent.

Patented Dec. 2, 1919.

No Drawing.

Application filed July 2, 1919. Serial No. 308,188.

*To all whom it may concern:*

Be it known that we, AUSTIN GILBERT and CHARLES E. VANDER HOOF, citizens of the United States, residing at Hamilton, Butler 5 county, Ohio, have invented certain new and useful Improvements in Sealing Compositions for Cans, of which the following is a specification.

This invention, pertaining to the sealing 10 of cans, relates to a composition to be employed in the sealing of the lids of the cans to place.

Our sealing composition consists of:—

|               |       |                   |
|---------------|-------|-------------------|
| Crude rubber  | ----- | 6 pounds.         |
| Benzol        | ----- | About 38 gallons. |
| Beeswax       | ----- | About 2 pounds.   |
| Paraffin wax  | ----- | About 2 pounds.   |
| Talcum powder | ----- | About 7 pounds.   |

20 This composition we apply to the portion

of the lid which is to make contact with the flange of the can body. The evaporation of the benzol leaves a substantially dry coating, leaving the lid in condition for future application to the can-body. When the lid 25 is applied to the can-body then the skirting is forcibly turned up under the flange, causing the composition to be compressed between the lid and the flange of the can-body.

30 We claim:—

A sealing composition for cans consisting of crude rubber, benzol, beeswax, paraffin wax, and talcum powder, in the proportions combined substantially as set forth.

AUSTIN GILBERT.  
CHARLES E. VANDER HOOF.

Witnesses:

ALLEN ANDREWS,  
M. S. BELDEN.